

## UNITED STATES PATENT OFFICE

2,564,268

## CATALYTIC OIL CRACKING

Eugene V. Mathy and Carl J. Helmers, Bartlesville, Okla., assignors to Phillips Petroleum Company, a corporation of Delaware

No Drawing. Application November 10, 1947,  
Serial No. 785,199

3 Claims. (Cl. 196—52)

1

This invention relates to an improved process for the catalytic cracking of hydrocarbon oils to produce a high yield of high octane gasoline motor fuel. In another aspect it relates to a process for the catalytic cracking of hydrocarbon oils in which the yield of gaseous by-products is low. In another aspect it relates to such a process in which the amount of carbon deposition is low. In still another aspect, it relates to an improved catalyst and a method of preparation of same.

In the production of gasoline motor fuel from petroleum, a small amount may be obtained by simple fractionation. Since gasoline motor fuel is the petroleum product in greatest demand, efforts are being constantly made to devise methods or processes to produce this gasoline motor fuel in greater quantities. The processes presently giving best results rely on the conversion of higher boiling hydrocarbon oils into low-boiling gasoline motor fuels in a system employing a catalyst in the conversion zone. This catalyst may be used in a fixed bed or a fluidized system. The search for improved catalysts is being pushed constantly and probably will never be ended.

Since the cracking reactions and catalyst regeneration are carried out at temperatures of 800—1400° F., a good catalyst must be able to withstand exposure to high temperatures without serious impairment of efficiency. The process must allow a high throughput of high-boiling point oil and return a high yield of high octane gasoline. The amount of dry gas (propane and lighter hydrocarbons) formed should be low. As carbon from the cracking builds up on the catalyst, the catalytic activity drops, and the catalyst must be taken out of service for regeneration when the activity drops to a certain predetermined level. Therefore, it is desirable that the rate of carbon deposition be as low as is consistent with economical operation of the process. However, the carbon deposition increases with an increase in the space velocity at constant conversion or with an increase in per cent conversion at constant space velocity, so an optimum balance between these important factors must be maintained.

We have found that catalysts having a high order of activity for converting high-boiling hydrocarbon oils into gasoline with a superior octane rating may be prepared by impregnating a solid, absorbent, catalytically active material with a mixed  $B_2O_3$  and  $P_2O_5$  promoter.

The principal object of our invention is to provide an improved process for the catalytic conversion of high-boiling petroleum oils into high

2

octane gasoline motor fuels at a high yield through the use of the catalyst comprising a major constituent selected from the group consisting of bauxite, fuller's earth, acid treated 5 montmorillonite clay, and the synthetically prepared alumina, silica, and silica-alumina gels supporting a minor proportion of boric oxide and phosphorus pentoxide.

Another object of our invention is to provide a process for the catalytic conversion of high-boiling point petroleum oils into high octane gasoline motor fuels at a high yield and without forming an unduly high amount of dry gas.

Another object of our invention is to provide 15 a process for the catalytic conversion of high-boiling point petroleum oils into high octane gasoline motor fuels at a high yield and without depositing an unduly high amount of carbon.

Another object of our invention is to provide 20 a process for the catalytic conversion of high-boiling point petroleum oils into high octane gasoline motor fuels, in which process, the catalyst is maintained at high activity and high efficiency for longer periods.

Another object is to provide a new and improved catalyst for the conversion of hydrocarbon oils into high octane gasoline.

Another object is to provide a method of preparing said catalyst.

Numerous other objects and advantages of our 30 invention will be apparent to those skilled in the art upon reading the following specification and the accompanying claims.

## OPERATIONS

35

Our invention is an improved process for the catalytic conversion of high-boiling point petroleum oils into high octane gasoline motor fuel wherein use is made of an improved catalytic 40 mass comprising a major constituent selected from the group consisting of bauxite, fuller's earth, acid treated montmorillonite clay, and the synthetically prepared alumina, silica and silica-alumina gels impregnated with minor 45 amounts of boric oxide and phosphorus pentoxide. While less amounts give some conversion, and greater amounts give similar conversion but are not as economical, we prefer to employ in this catalyst from 0.1 to 10% by weight of boric oxide and from 0.1 to 10% by weight of phosphorus pentoxide.

In its operation, the high-boiling point oil is substantially vaporized in a preheater, passed into a catalytic reactor where it is contacted with 55 the catalyst for the desired time, and then passed

into a conventional fractionating and separating system.

Before the petroleum oil is introduced into the high temperature section of the preheater, we prefer to dilute it with about 60 pounds of steam per barrel of oil. Any other diluent gas may be used or this dilution may be omitted entirely. The charge is vaporized and superheated with as little thermal decomposition as possible to a temperature in the range of 850-1100° F. A pressure of 10-300 pounds per square inch gauge at the preheater outlet is preferred.

The vaporized petroleum oil is passed from the preheater into the catalytic reactor where it contacts the catalytic mass at a space velocity of from 0.1-10 liquid volumes of petroleum oil per volume of catalytic mass per hour. The amount of conversion is partially controlled by the length of time the oil is exposed to the catalyst. However, if the velocity is low, the process is uneconomical because the total product will be low and the rate of carbon deposition increases. If

the initial high activity of the catalyst. It was calculated that the promoter content was 1.05 weight per cent of  $P_2O_5$  and 1.05 per cent of  $B_2O_3$ .

5 A catalyst of bauxite containing  $P_2O_5$  alone in the amount of 1.4 weight per cent and one containing  $B_2O_3$  alone in the amount of 2.0 weight per cent were prepared in a similar manner.

#### EXAMPLE II

10 The four catalysts prepared in Example I were tested in a fixed bed hydrocarbon cracking system charged with an oil having a boiling point essentially above that of gasoline. A catalyst temperature of 1015° F., a pressure of 85 pounds per square inch gauge, and an operating period of 3 hours were used. The space velocities, measured in terms of liquid volumes of oil per volume of catalyst per hour, were held constant for all tests. The results are shown in Table I. 15 The activity index is the comparison of the per cent conversion obtained with each catalyst compared with that of the original bauxite.

Table I

|                             | Bauxite | Bauxite + 2.0% $B_2O_3$ | Bauxite + 1.4% $P_2O_5$ | Bauxite + 1.05% $B_2O_3 + 1.05\% P_2O_5$ |
|-----------------------------|---------|-------------------------|-------------------------|------------------------------------------|
| Space Velocity.....         | 1.8     | 1.8                     | 1.8                     | 1.8                                      |
| Per Cent Conversion.....    | 51.2    | 63.9                    | 52.3                    | 56.5                                     |
| Dry Gas, wt. per cent.....  | 12.9    | 13.4                    | 12.8                    | 14.1                                     |
| Butanes, vol. per cent..... | 6.2     | 7.4                     | 7.8                     | 8.1                                      |
| Carbon, wt. per cent.....   | 1.8     | 2.0                     | 2.8                     | 3.4                                      |
| Gasoline:                   |         |                         |                         |                                          |
| Yield, vol. per cent.....   | 35.0    | 38.3                    | 34.4                    | 38.2                                     |
| ASTM Octane No.....         | 75.6    | 76.6                    | 77.2                    | 76.8                                     |
| Bromine No.....             | 91      | 96                      | 88                      | 81                                       |
| Activity Index.....         | 100     | 105                     | 102                     | 110                                      |

the space velocity is too high, the per cent conversion is too low. We prefer a space velocity of about 0.5 to 2.0 liquid volumes of oil per volume of catalyst per hour. We prefer to use a top bed catalyst temperature of 950-1000° F. and a catalyst case pressure of 10-95 pounds per square inch gauge. The pressure may be varied over a fairly wide range with very little effect on the conversion yields.

For our catalyst, any solid, catalytically active adsorbent material of the nature of bauxite, fuller's earth, acid treated montmorillonite clay, or a synthetically prepared silica, alumina, or silica-alumina gel which material has been impregnated with a minor proportion of boron trioxide and phosphorus pentoxide as a combination promoter may be used.

The effluent gases from the catalytic reactor are led into a separator where the gasoline motor fuel, dry gas, and butanes are removed. If desired, the high-boiling fraction may be recycled through the system by introducing it back into the preheater. The following examples serve to illustrate further the advantages of our invention.

#### EXAMPLE I

Samples of our catalysts were prepared as follows:

A portion of bauxite containing less than 3 per cent of iron and having a particle size of 8-14 mesh was calcined at a temperature of 700-900° F. for a period of about 10 hours to reduce the water content below 5 per cent.

A 250 gram sample of the calcined bauxite was 70 soaked for 1 hour in 250 ml. of solution containing 10.1 grams of  $H_3PO_4$  and 11.7 grams of  $H_3BO_3$ . The mass was then drained for 1 hour, air dried for 3 days, oven dried at 432° F. for 20 hours, and heat treated for 168 hours at 1500° F. to "kill" 75

The bauxite impregnated with  $B_2O_3$  and the bauxite impregnated with  $P_2O_5$  catalyst has a higher activity index than the untreated bauxite. The catalytic effect of our catalyst is more than the combined effect produced by  $B_2O_3$  and  $P_2O_5$  separately.

#### EXAMPLE III

45 Another comparison was made using a high grade bauxite and the same bauxite impregnated with  $B_2O_3$  and  $P_2O_5$  in minor amounts for cracking a virgin gas oil. The octane numbers were run on the product gasoline clear and with 1 50 and 3 ml. of tetraethyl lead per gallon of gasoline. The operating conditions and results are shown in Table II.

Table II

|                                     | Beauxite | Bauxite + $B_2O_3 + P_2O_5$ |
|-------------------------------------|----------|-----------------------------|
| Pressure.....                       | 85       | 85                          |
| Temperature, ° F.....               | 980      | 980                         |
| Conversion, Vol. Per Cent.....      | 52       | 54                          |
| Gasoline:                           |          |                             |
| Yield, Vol. Per Cent.....           | 38.3     | 35.7                        |
| Bromine No.....                     | 74       | 70                          |
| Cycle Stock, Vol.....               | 48.0     | 45.4                        |
| Dry Gas, wt. Per Cent.....          | 9.8      | 11.5                        |
| Tests for tetraethyl lead response: |          |                             |
| ASTM Octane Numbers—                |          |                             |
| 0 ml. TEL per gal.....              | 74.1     | 76.5                        |
| 1 ml. TEL per gal.....              | 78.5     | 80.0                        |
| 3 ml. TEL per gal.....              | 81.8     | 82.7                        |
| Research Octane Numbers—            |          |                             |
| 0 ml. TEL per gal.....              | 82.3     | 86.3                        |
| 1 ml. TEL per gal.....              | 88.7     | 92.0                        |
| 3 ml. TEL per gal.....              | 92.4     | 94.1                        |

The higher conversion obtained by using our catalyst more than compensates for the slightly lower gasoline yield. The superiority of our catalyst is clearly shown in the higher octane rating of the gasoline produced.

From the foregoing examples, it is apparent that this process has many advantages. The catalytic activity is not impaired by prolonged exposure to high temperatures. When our catalyst is employed a gasoline of a high octane rating is produced. The low rate of carbon deposition means prolonged life of the catalyst at high activity. Due to the high catalytic activity as reflected in the high conversion ratio, our catalyst permits a higher space velocity or throughput than is possible with the other catalysts tested. This means that more high-boiling point petroleum oil may be processed in less time and with a high yield of high octane gasoline motor fuel.

In the practicing of this invention it is obvious that variations in the arrangement may be made without invention. For instance, instead of the fixed-bed catalyst described in the examples, a fluidized bed may be used. This invention embraces such other obvious variations and modifications as come within the scope thereof. This invention is limited only by the following claims.

Having fully described our invention, we claim:

1. A process for the conversion of hydrocarbon oils to produce a high octane gasoline which comprises passing said oil at a cracking temperature and pressure through a cracking zone containing an active catalyst comprising bauxite supporting impregnated on its surface 1 to 10 weight per cent of phosphorus pentoxide and boron trioxide as such and maintaining said hydrocarbon oil in contact with said catalyst for a period of time sufficient to obtain the desired conversion thereof.

2. A process for cracking hydrocarbon oils which comprises contacting the said hydrocarbon oil at a temperature of 800° F. to 1400° F., a pressure between 10 and 300 pounds per square inch

gauge, and a space velocity of from 0.1 to 10 volumes of liquid charge per volume of catalyst per hour with an active catalytic mass comprising bauxite as a major constituent supporting impregnated thereon as such 0.1 to 10 weight per cent of boron trioxide and 0.1 to 10 weight per cent of phosphorus pentoxide.

3. A catalyst for the cracking of hydrocarbon oils prepared by calcining bauxite at about 900° F. to reduce the water content below 5 per cent, soaking said calcined bauxite in an aqueous solution of boric and phosphoric acids, drying this catalytic mass and finally heat treating it at about 1500° F. for a period of time sufficient to produce a catalytic mass containing less than 5 per cent of water and minor amounts of boric oxide and phosphorus pentoxide impregnated and supported as such on bauxite.

EUGENE V. MATHY.  
CARL J. HELMERS.

#### REFERENCES CITED

The following references are of record in the file of this patent:

#### UNITED STATES PATENTS

| Number       | Name     | Date          |
|--------------|----------|---------------|
| 2,109,866    | Moser    | Mar. 1, 1938  |
| 2,341,363    | Connolly | Feb. 8, 1944  |
| 30 2,398,819 | Cook     | Apr. 23, 1946 |
| 2,441,493    | Krug     | May 11, 1948  |
| 2,443,402    | Schulze  | June 15, 1948 |
| 2,480,672    | Plank    | Aug. 30, 1949 |

#### OTHER REFERENCES

- 35 Mellor, "Comprehensive Treatise on Inorganic and Theoretical Chemistry," vol. 5, page 147.  
Handbook of Chem. & Physics "Hagman and Lange," 16th edition, page 198.